

## UNITED STATES PATENT OFFICE

WALTER PFAU, OF COLOGNE-MUHLHEIM, GERMANY, ASSIGNOR TO EMIL BAGGLI, OF ZURICH, SWITZERLAND, AND EDWIN BURGER, OF GISIKON NEAR ROOT, SWITZERLAND

## METHOD OF PRODUCING BERYLLIUM-ALUMINIUM ALLOY

No Drawing. Application filed March 5, 1932, Serial No. 597,089, and in Germany March 14, 1931.

This invention relates to a method of producing beryllium-aluminium alloys.

Various methods of producing such alloys are known, one of them consisting in obtaining the beryllium and aluminium metals separately and then melting them together. However, owing to the high fusing temperatures required, heavy oxidation of the metals is unavoidable which renders the product useless. Another known process reduces the mixed metallic salts or oxides of beryllium and aluminium to a metal alloy in a thermochemical manner, but the alloys produced in this way are very impure and, furthermore, do not ensue in compact form.

For technical purposes, electrolysis is therefore employed to produce beryllium-aluminium alloys, and in this connection it has been proposed already to use as electrolyte a mixture of molten double salts of these metals. The general practice has been in this respect to produce beryllium salt separately from aluminium salt in the form of basic beryllium fluoride or oxyfluoride and to subject it in mixture with a suitable aluminium salt, such as the fluoride, to electrolysis while adding alkaline and alkaline earth fluorides.

The prevailing practice carefully avoided to subject a basic fluoride or oxyfluoride to electrolysis, which contained aluminium besides beryllium, since it was generally assumed that a suitable electrolyte could be produced only from separately obtained basic beryllium fluoride or oxyfluoride.

According to the invention, beryllium-aluminium alloys can be produced by simultaneously and jointly converting the metallic oxides of beryllium and aluminium contained in the beryl ores (beryl =  $3\text{BeO} \cdot \text{Al}_2\text{O}_3 \cdot 6\text{SiO}_2$ ), by suitable treatment, into basic fluorides or oxyfluorides and subjecting the salts thus gained, together with conducting salts, to electrolysis of fused electrolytes, in which case, as many experiments have shown, a beryllium-aluminium alloy will be precipitated on the cathode without trouble.

Compared with existing methods, the new process involves a considerable economic advantage in so far as the same operations or steps will instantly yield the requisite double

salts of beryllium and aluminium by the simple application of hydrofluoric acid.

## Example

1 kilogram of beryllium ore is finely ground and then mixed with 1 kilogram of sodium fluosilicate whereupon the mixture is heated for several hours. To produce the double basic fluorides the mixture is leached out with acidified water which will then contain in dissolved form the double fluorides of beryllium-sodium and aluminium-sodium. The liquid is then decanted and treated with ammonia to precipitate the hydroxides of beryllium and aluminium which are separated by filtration and then treated with hydrofluoric acid whereupon, after evaporation, the basic fluorides or oxyfluorides of beryllium and aluminium will jointly ensue in the proportion of 80% basic beryllium fluoride or oxyfluoride and 20% basic aluminium fluoride. In this composition the metal contents amount to approximately 18% beryllium and approximately 6% aluminium, so that electrolysis will produce a beryllium-aluminium alloy which has an aluminium content of about 25%.

The electrolysis is preferably carried out in the following manner. Into a suitable graphite crucible 200 grams of sodium fluoride are placed first on account of easier fusibility. The crucible is then heated from without and gradually filled with 1 kilogram of the double basic fluorides or oxyfluorides of the composition described together with 1 kilogram of barium chloride. Electrolysis is begun at a temperature of approximately 1200° centigrade, the crucible being used as anode while a water-cooled iron pipe closed below and immersed in the melt serves preferably as cathode. The electrolysis can be carried out at about 70 volts and a current intensity of 100 amperes corresponding to a current density of about 40 amperes per  $\text{cm}^2$  on the cathode, whereupon a beryllium-aluminium alloy will settle on the cathode in compact form or as coating. It is however more advantageous to operate with considerably higher current densities, up to ten times the values given above, since during the evapora-

tion in connection with electrolysis more rapid metal separation will lead to better metal yield.

I claim:—

- 5 1. A method of producing beryllium-aluminium alloys in compact form or as coating by electrolysis of fused electrolytes, which consists in employing as electrolyte a melt of basic fluorides of beryllium and aluminium 70 jointly obtained from the ores and adding thereto halogen salts of the alkaline and alkaline earth metals to act as conducting salts.
- 10

2. A method of producing beryllium-aluminium alloys in compact form or as coating by electrolysis of fused electrolytes, which consists in employing as electrolyte a melt of basic oxyfluorides of beryllium and aluminium jointly obtained from the ores and adding thereto halogen salts of the alkaline and alkaline earth metals to act as conducting salts.

WALTER PFAU.

75

15

80

20

85

25

90

30

95

35

100

40

105

45

110

50

115

55

120

60

125

65

130